

1,318,630.

S. A. WAUGH,  
METHOD OF MANUFACTURING GRINDING WHEELS,  
APPLICATION FILED MAY 3, 1917.

Patented Oct. 14, 1919.

Fig. 1.



Fig. 2.



Attest:

*S. A. Waugh*

Inventor:  
by *Samuel A. Waugh,*  
*Ernest G. Rincon*  
his Atty.

# UNITED STATES PATENT OFFICE.

SAMUEL A. WAUGH, OF REVERE, MASSACHUSETTS, ASSIGNOR TO REVERE RUBBER COMPANY, A CORPORATION OF RHODE ISLAND.

## METHOD OF MANUFACTURING GRINDING-WHEELS.

1,318,630.

Specification of Letters Patent.

Patented Oct. 14, 1919.

Application filed May 3, 1917. Serial No. 166,135.

To all whom it may concern:

Be it known that I, SAMUEL A. WAUGH, a citizen of the United States, residing in Revere, county of Suffolk, and State of Massachusetts, have invented certain new and useful Improvements in Methods of Manufacturing Grinding-Wheels, of which the following is a full, clear, and exact description.

10 This invention relates to grinding wheels and methods of manufacturing same, more particularly to grinding wheels for finishing relatively soft surfaces, such for instance as rubber covered iron rolls. The object of this invention is to produce a grinding wheel having the desired abrasive surface and great lasting qualities, which may be run at high speed without danger of exploding, and which is capable of receiving 20 a new abrasive surface with a minimum of expense and equipment.

Heretofore it has been customary in the manufacture of grinding wheels to mix the abrasive material with a suitable binder to 25 form a plastic mass, then shape the wheel therefrom in suitable molds or the like, and finally compact it by hydraulic pressure. By this invention I provide a method of manufacturing grinding wheels wherein 30 the necessity of mixing the abrasive material with the binder is obviated, and in which the grinding surface is applied to its core or form without the use of molds, presses or the like.

35 For a clearer understanding of this invention, reference is made to the following specification and the accompanying drawing in which—

Figure 1 is a perspective view, partly 40 broken away of a grinding wheel made according to this invention, and

Fig. 2 is a cross sectional view of the grinding surface of the same.

A suitable metal wheel or pulley 1 is finished to the required diameter and its peripheral surface roughened in any desired manner, as by cutting threads thereon. To the thus roughened surface 2, I apply a coating of rubber solution or cement 3, the 45 solution having compounded with it a suitable vulcanizing agent such as sulfur. The coating of solution 3 is then permitted to dry for a short period and a stratum 4 of comminuted abrasive superposed thereon. 50 This I accomplish preferably by rolling the

wheel in the abrasive, which adheres to the cemented surface. A second coating 5 of rubber solution is then applied over the abrasive and dried as in the first instance. To this a second stratum 6 of abrasive is 60 applied and so on with the alternate layers 7, 8, 9 and 10 of rubber and abrasive respectively or until the material reaches the required thickness.

The number of strata indicated provides 65 an abrasive surface of sufficient depth (about one eighth inch) for most purposes, but of course a greater or less number may sometimes be desirable, the exact number varying according to the thickness of the 70 rubber solution, the total depth desired, etc.

Having applied the desired amount of rubber and abrasive, the whole is allowed to dry until all of the solvent in the rubber has 75 evaporated. This usually requires about three days. The wheel is then tightly wrapped to maintain the material in place during vulcanization. I have found that a satisfactory cure is accomplished by subjecting the wheel to a temperature of approximately 280° F. for about five hours but this may be varied according to the amount of vulcanizing medium in the compound. To prevent possible displacement 80 of the abrasive surface after vulcanization the wrappings are left in place for at least a day after removal of the wheel from the vulcanizing chamber. They are then removed, and after an additional ageing period of about two days the wheel is ready 85 for use.

It may be seen that the above method is of particular advantage in that it obviates the necessity of providing molds and presses to 90 shape and compact the abrasive wheel, also in that it obviates the step of mixing the abrasive compound in mills or other apparatus.

I have found that the abrasive surface 95 produced by my method of manufacture has greater lasting qualities than in any of the types of grinding wheels heretofore provided for grinding relatively soft surfaces such as rubber covered rollers.

When the abrasive surface of a wheel 100 built according to my method has worn away, it can of course, be easily resurfaced by applying additional strata thereto by the same method as above outlined.

105 Wheels manufactured according to this 110

invention do not explode when run at high speeds and their use therefore eliminates all danger of injury to workmen in this regard, a danger which is very serious when 5 using the ordinary type of grinding wheel.

Having thus described my invention, what I claim and desire to protect by Letters Patent is:

1. The method of manufacturing grinding wheels which consists in coating the surface of a metal core with rubber in a solvent and a vulcanizing agent, applying an abrasive to the tacky surface of the rub-

ber, reducing the solvent, repeating said steps until the desired strata have been applied upon the core, and subjecting the article to vulcanization.

2. The method of manufacturing grinding wheels which consists in applying to the surface of a metal core alternate layers of vulcanizable rubber solution and abrasive material, reducing the solvent by volatilization, and vulcanizing the article.

Signed at Chelsea, Mass., this 30th day of April, 1917.

SAMUEL A. WAUGH.